

# United States Patent

[11] 3,634,1

[72] Inventors **John G. Cutton**  
Board Township, Mahoning County;  
**George A. Welsch, Jr.**, Youngstown, both of  
Ohio  
[21] Appl. No. **840,456**  
[22] Filed **July 9, 1969**  
[45] Patented **Jan. 11, 1972**  
[73] Assignee **United States Steel Corporation**

[54] **FREE-MACHINING STEEL, ARTICLES THEREOF  
AND METHOD OF MAKING**  
6 Claims, No Drawings

[52] U.S. Cl..... **75/123 D,**  
75/123 G, 75/123 H, 75/123 L, 75/126 F, 75/126  
K, 75/126 L, 75/129, 75/130.5

[51] Int. Cl..... **C22c 39/26,**  
C22c 39/44, C22c 39/54

[50] Field of Search..... **75/123,**  
129, 123 H, 126 F, 128.8

[56] **References Cited**  
UNITED STATES PATENTS  
2,157,673 5/1939 Ridgely ..... 7:  
2,182,758 12/1939 Harder ..... 7:  
3,169,857 2/1965 Rathke ..... 7:  
*Primary Examiner—L. Dewayne Rutledge*  
*Assistant Examiner—Joseph E. Legru*  
*Attorney—John R. Pegan*

**ABSTRACT:** Improved free-machining, resulfurized  
repophosphorized carbon and low alloy steels, especially  
barrel steels, method of making the same, and articles the  
containing 0.015 to 0.15 weight percent zirconium for  
proved chemical and structural homogeneity, enhanced  
workability and hot-rolled surface quality, increased strength  
and superior hardness uniformity.

## FREE-MACHINING STEEL, ARTICLES THEREOF AND METHOD OF MAKING

## BACKGROUND OF THE INVENTION

Many of the standard grades of carbon steels are available with larger than usual amounts of sulfur (normally 0.045 to 0.05 percent maximum in plain carbon steels) and phosphorus (normally 0.035 to 0.04 percent maximum in plain carbon steels) in order to provide the free-machining benefits derivable from increased percentages of one or both of these elements.

The so-called "resulfurized" and "rephosphorized" carbon steels embraced within the AISI series 1100 and 1200 steels conform to the following table I compositional range, by weight percent:

TABLE I

|            |                                                         |
|------------|---------------------------------------------------------|
| carbon     | 0.08 to 0.55%                                           |
| manganese  | 0.30 to 1.65%                                           |
| silicon    | up to 0.30%                                             |
| sulfur     | 0.08 to 0.35%                                           |
| phosphorus | up to 0.12%<br>(over 0.04 for<br>rephosphorized steels) |
| iron       | balance, except for<br>incidental impurities.           |

Resulfurized and rephosphorized alloy steels are also known to the art, for example, low alloy steels which, while conforming to the above table I compositional range, are strengthened or otherwise modified by the incorporation of additional alloying elements such as chromium, nickel, molybdenum, copper, vanadium, titanium or boron. Illustratively, such steels may contain chromium up to about 1.5 percent, nickel up to about 3.8 percent, molybdenum up to about 0.60 percent, copper up to 1.00 percent, vanadium up to about 0.30 percent, columbium up to about 0.05 percent, titanium up to about 0.03 percent, and boron up to about 0.006 percent. Reference herein and in the appended claims to "low alloy" steels is intended to include steels within the table I compositional range with one or more additional alloying elements as aforesaid up to a total of such alloying element additions of about 4 percent. Like the mentioned carbon steels, such low alloy steels may also contain lead, in amount of about 0.15 to 0.35 percent for machinability enhancement. Exemplary of the resulfurized low alloy steels of the prior art are steels having compositions within the range: 0.47 to 0.55 percent carbon, 0.95 to 1.30 percent manganese, 0.60 to 0.90 percent chromium, 0.06 to 0.10 percent sulfur, and balance substantially iron.

The large percentages of sulfur and/or phosphorus in prior art free-machining steels tend to the formation of relatively large sulfide inclusions, or segregates high in sulfur and phosphorus contents, whereby the full machinability benefits of these elements are not realized and internal soundness and microstructural homogeneity of ingots of such steels and products made therefrom are adversely affected. Moreover, such high-sulfur, high-phosphorus prior art steels are prone to hot shortness, with resultant difficulties in hot working, and hot-rolled products thereof commonly present surfaces of low quality with many seams resulting in poor mill yields.

Attempts have been made in the past to correct these deficiencies of such free-machining steels, for example, by addition of alloying elements, such as boron (Murphy U.S. Pat. No. 2,388,214) to inhibit sulfur segregation. Boron, however, even in small amounts is very potent in its effect on hardenability of steels, and even slight inhomogeneities in boron-containing steels intended for critical machining applications sometimes result in large variations in hardness and hence in variable machining characteristics. Further, boron is rendered largely ineffective if added to other than fully aluminum deoxidized steels.

## SUMMARY OF THE INVENTION

The present invention provides a method for the increasing mill yield in the production of new and improved resulfurized and rephosphorized free-machining steels which exhibit enhanced hot rollability, improved hot-rolled surface quality and improved ingot soundness and structure, including decreased segregation of constituent elements, especially sulfur, phosphorus and carbon. The new steels also show increased yield and tensile strengths and more uniform hardness as compared to prior art steels. In a preferred embodiment these advances are achieved by the addition of at least at 0.015 percent, preferably 0.015 to 0.15 percent, especially 0.015 to 0.05 percent, zirconium to a base composition comprising, by weight percent:

TABLE II

|    |            |                                               |
|----|------------|-----------------------------------------------|
| 20 | carbon     | 0.30 to 0.45%                                 |
|    | manganese  | 0.70 to 1.0%                                  |
|    | silicon    | 0.10% maximum                                 |
|    | sulfur     | 0.08 to 0.15%                                 |
|    | phosphorus | 0.07 to 0.12%                                 |
| 25 | iron       | balance, except for<br>incidental impurities. |

## DESCRIPTION OF THE INVENTION

Zirconium is known in the metallurgical arts as a useful addition to special purpose steels, for example, deep-draw steels and low alloy, high-strength steels, for its deoxidizing and grain refining effects. Selmi et al. U.S. Pat. No. 2,200,350 teaches the addition of 0.10 to 0.15 percent zirconium to low alloy steels of good deep-drawing properties, high fatigue resistance and freedom from strain and quench aging. Bidwell U.S. Pat. No. 2,840,872 discloses high-strength, low alloy steels containing 0.03 to 0.11 percent zirconium as a deoxidizer added to the mold or ladle in the form of a zirconium and aluminum-containing material. Such known metallurgical effects of zirconium as an alloying additive to steels is recognized in the *Metals Handbook*, vol. 1, page 90, 8th edition, 1961, published by the American Society for Metals. Crafts, U.S. Pat. No. 2,280,283 discloses the addition of zirconium to titanium, cerium, hafnium, thorium, vanadium, columbium, tantalum or uranium, in amount of 0.03 to 1.0 percent, further enhance deep hardenability conferred by one or combination of the elements boron, silicon, molybdenum, tungsten, chromium or nickel. Crafts, too, recognizes the grain-refining effect of the several elements of the above-mentioned zirconium-containing group of elements, but derives the additional deep-hardenability effect from an addition larger than that required for grain refining.

We have now found that zirconium, when added in certain restricted amounts to resulfurized and rephosphorized free-machining carbon and low alloy steels, contributes to such steels certain new and beneficial properties and effects above and beyond those heretofore known to or practiced by the metallurgical arts.

Many free-machining steels containing high percentages of sulfur and phosphorus are difficult to hot roll, and the hot-rolled surface is of poor quality. Exemplary of such steels is AISI grade 1140, having a composition essentially as given in table II above. Such steels, furthermore, when cast, commonly are productive of ingots having widely varying chemical compositions, e.g., from center to surface of the ingot, together with a significant microstructural heterogeneity. The latter characteristic is particularly evidenced by the presence in ingots of such steels of large sulfide inclusions and sulfur- and phosphorus-containing segregates. Still further, ingots of such steels, cast by usual steel mill practices, exhibit a high degree of subsurface porosity. These ingot defects commonly contribute to high product loss and low semifinished mill yields, e.g., on the order of 60 percent.

Illustrative of the present invention, a heat was made of a gun barrel quality steel of composition in general accordance with AISI grade 1140 steel, but modified with a small alloying addition of chromium. Ingots of such heat were poured directly, and to another part of such heat a mold addition of zirconium was made, in the form of 10 pounds of an alloy (1 pound of zirconium per ton of steel) which analyzed to the following approximate composition, by weight percent:

TABLE III

|           |        |
|-----------|--------|
| silicon   | 51.17% |
| zirconium | 39.23% |
| iron      | 9.10%  |
| carbon    | 0.44%  |

he ingots were 21×23 inches in cross section and weighed about 7,900 pounds each. The ladle analyses of these steels were as given in the following table:

TABLE IV

| Heat Number | Ingot Number | Type            | Composition, weight percent |     |     |     |     |     |      |      |                       |
|-------------|--------------|-----------------|-----------------------------|-----|-----|-----|-----|-----|------|------|-----------------------|
|             |              |                 | C                           | Mn  | Si  | S   | P   | Cr  | Al   | Zr   | Fe                    |
| D300        | 8            | "Regular"       | .38                         | .89 | .07 | .12 | .09 | .18 | .002 | .003 | Balance. <sup>1</sup> |
| K-0114      | 7            | "Zr-containing" | .40                         | .93 | .16 | .12 | .10 | .13 | .002 | .027 | Do.                   |

Except for usual steel-making impurities.

Such ingots were hot-rolled to 2½-inch-square billets, during which it was observed that the KX-0114 hot-rolled product had a good, smooth surface, as contrasted with the "regular" 41D300 product, the surface of which was highly pitted.

Three-eighth-inch-diameter drillings were made on the billet cross sections at center and midway between center and side surface, and the drilling chips were analyzed, with results as shown in table V:

TABLE V

got No. 7 (KX-0114 zirconium-treated, from regular parent heat 41D300)

| Sample Number | Ingot Location | Composition, weight percent |     |     |     |      |
|---------------|----------------|-----------------------------|-----|-----|-----|------|
|               |                | C                           | Si  | S   | P   | Zr   |
| center        | Top, No. 1     | .41                         | .13 | .14 | .11 | .054 |
| midway        | 1.             | .40                         | .12 | .12 | .11 | .034 |
| center        | Top, No. 2     | .43                         | .12 | .16 | .14 | .034 |
| midway        | 2.             | .40                         | .12 | .12 | .11 | .038 |
| center        | Top, No. 3     | .42                         | .11 | .15 | .13 | .042 |
| midway        | 3.             | .41                         | .11 | .13 | .11 | .040 |
| center        | Bottom         | .30                         | .11 | .09 | .09 | .066 |
| midway        |                | .33                         | .10 | .10 | .09 | .047 |

Average percent Zr..... 0.044

| Ingot No. 8 (regular heat 41D300) |            |     |     |     |     |      |
|-----------------------------------|------------|-----|-----|-----|-----|------|
| center                            | Top, No. 1 | .59 | .10 | .28 | .22 |      |
| midway                            | 1.         | .43 | .10 | .13 | .13 |      |
| center                            | Top, No. 2 | .47 | .09 | .22 | .19 |      |
| midway                            | 2.         | .37 | .10 | .11 | .11 |      |
| center                            | Top, No. 3 | .41 | .08 | .14 | .13 | None |
| midway                            | 3.         | .38 | .09 | .11 | .11 |      |
| center                            | Bottom     | .28 | .07 | .08 | .09 |      |
| midway                            |            | .30 | .06 | .08 | .09 |      |

From the chemical segregation data of table V, it is seen that the zirconium-treated product was significantly less segregated, as regards carbon, sulfur and phosphorus, than the untreated product, thus:

TABLE VI

| Ave. difference (wt.% × 10 <sup>2</sup> ) between center and midway analysis (from table V) |     |      |
|---------------------------------------------------------------------------------------------|-----|------|
| C                                                                                           | S   | P    |
| Untreated steel                                                                             | 2.0 | 2.25 |
| Zr-treated steel                                                                            | 7.5 | 7.25 |

Macroexamination was made of the first (top) three and the last (bottom) billet produced from each of the foregoing ingots 7 and 8, from which it was observed that the zirconium-containing billets showed little or no visible segregation or subsurface porosity, whereas the zirconium-free billets showed heavy center segregation and extensive subsurface porosity. Despite the inherent deoxidizing capacity of zirconium, the relatively small amount added was such that the steel behaved as a semikilled steel, and no pipe was observed on the top billets of the No. 7 ingot.

The billets above mentioned were further reduced by hot rolling to 1-inch rounds. To this point, total mill yields were:

TABLE VII

| Percent Mill Yield         |        |
|----------------------------|--------|
| Zirconium-containing steel | 81.65% |
| Zirconium-free steel       | 64.87% |

Micro examination of the respective 1-inch round samples showed a slight grain refinement by the McQuaid Ehn grain size test,

TABLE VIII

| Grain Size                 |                             |
|----------------------------|-----------------------------|
| Zirconium-containing steel | Duplex: 90% 6 to 8; 10% 2-4 |
| Zirconium-free steel       | 2-4 (ave. 3).               |

and a more evenly distributed microstructure, the zirconium-containing product being essentially free of large pearlite areas which were prominent in the nontreated steel.

Strength and ductility of duplicate test specimens of the foregoing table IV comparison steels were as given in table IX:

TABLE IX

| Steel   | Test | 0.2% offset Y.S., p.s.i. |        | U.T.S., p.s.i. | Percent elongation, in 2 inches | R.A., percent |
|---------|------|--------------------------|--------|----------------|---------------------------------|---------------|
|         |      | 1                        | 2      |                |                                 |               |
| Zr-free |      | 50,930                   | 87,120 | 32.0           | 52.4                            |               |
|         |      | 51,180                   | 84,380 | 30.0           | 55.8                            |               |
|         |      | 58,420                   | 98,100 | 24.0           | 42.2                            |               |
|         |      | 56,920                   | 94,110 | 24.0           | 43.1                            |               |

Thus, the zirconium-containing steel exhibited a significant strength increase while retaining excellent ductility.

Hardness tests were made across the cross section of the 1-inch round specimens, with results as set forth in table X:

TABLE X.—HARDNESS, R<sub>B</sub>

| Steel         | Specimen Number | Distance from surface, inches |      |      |      |      |      |
|---------------|-----------------|-------------------------------|------|------|------|------|------|
|               |                 | 0                             | 0.15 | 0.30 | 0.50 | 0.30 | 0.15 |
| Zr-containing | 1               | 88                            | 89   | 90   | 90   | 90   | 89   |
|               | 2               | 88                            | 87   | 87   | 87   | 87   | 88   |
| Zr-free       | 1               | 88                            | 84   | 82   | 84   | 86   | 88   |
|               | 2               | 86                            | 85   | 83   | 85   | 86   | 87   |

As seen in table X, the specimens from the zirconium-containing steel, KX-0114, showed more uniform hardness from surface to center than did those of the zirconium-free steel, 41D300. Such superior hardness uniformity, together with the enhanced microstructural homogeneity exhibited by such new steels, is especially desirable in demanding machining applications such as long bore reaming, etc., wherein accurate cutting tool position is critical and is facilitated by uniformity of the steel being machined.

Further tests were carried out wherein varying amounts of zirconium, both in the form of zirconium-silicon alloy and zirconium metal, were added to gun barrel quality carbon steel (with added chromium).

TABLE XI

| Steel   | Ingot Number | Composition, weight percent (ladle analysis) |      |     |     |     |     |      |
|---------|--------------|----------------------------------------------|------|-----|-----|-----|-----|------|
|         |              | C                                            | Mn   | Si  | S   | P   | Cr  | Zr   |
| 52D524  | 2            | .35                                          | .94  | .05 | .12 | .09 | .16 | .003 |
| KX-0134 | 5            | .35                                          | .95  | .05 | .13 | .09 | .15 | .011 |
| KX-0135 | 6            | .35                                          | 1.03 | .05 | .14 | .10 | .15 | .014 |
| KX-0136 | 7            | .35                                          | 1.01 | .05 | .14 | .10 | .15 | .030 |
| KX-0137 | 8            | .35                                          | .98  | .05 | .14 | .10 | .15 | .026 |

<sup>1</sup> Except for normal steelmaking impurities.

As in the preceding test, the 21×23 inch cross section ingots were hot rolled to 2½-inch square billets, and ¾-inch drillings were made of the billets to determine chemical analyses at center and midway positions. Representative results are given in table XII.

TABLE XII

[Steel 52D524 (Ingot No. 2: Zr free)]

| Sample                                                          | Composition, weight percent |     |     |       |      |
|-----------------------------------------------------------------|-----------------------------|-----|-----|-------|------|
|                                                                 | C                           | Si  | S   | P     | Zr   |
| 2-1 center                                                      | .41                         | .05 | .14 | .10   | .001 |
| 2-1 midway                                                      | .44                         | .06 | .15 | .11   | .003 |
| 2-2 center                                                      | .48                         | .06 | .24 | .14   | .003 |
| 2-2 midway                                                      | .41                         | .06 | .15 | .11   | .002 |
| 2-3 center                                                      | .44                         | .07 | .21 | .13   | .002 |
| 2-3 midway                                                      | .38                         | .06 | .13 | .10   | .003 |
| 2-B center                                                      | .31                         | .07 | .11 | .08   | .002 |
| 2-B midway                                                      | .33                         | .06 | .11 | .09   | .003 |
| Average difference (×10 <sup>3</sup> ) =                        | 4.5                         |     | 4.5 | 2.0   |      |
| Steel KX-0135 (Ingot No. 6: 0.014% Zr, from parent heat 52D524) |                             |     |     |       |      |
| 6-1 center                                                      | .39                         | .08 | .22 | .16   | .011 |
| 6-1 midway                                                      | .40                         | .08 | .16 | .13   | .013 |
| 6-2 center                                                      | .46                         | .09 | .20 | .15   | .013 |
| 6-2 midway                                                      | .41                         | .09 | .15 | .12   | .015 |
| 6-3 center                                                      | .42                         | .08 | .16 | .13   | .018 |
| 6-3 midway                                                      | .38                         | .08 | .13 | .12   | .016 |
| 6-B center                                                      | .35                         | .08 | .12 | .11   | .017 |
| 6-B midway                                                      | .35                         | .08 | .12 | .11   | .017 |
| Average percent Zr                                              |                             |     |     | 0.148 |      |
| Average difference (×10 <sup>3</sup> ) =                        | 2.5                         |     | 3.5 | 1.75  |      |

<sup>1</sup> Bottom billet.

It is seen from table XII that as little as about 0.015 percent zirconium is effective in these free-machining steels to substantially diminish segregation of carbon, sulfur and phosphorus. Comparison with the data of table V, however, will show that somewhat greater amounts of zirconium, i.e. 0.044 percent or higher, provide a still greater effect on segregation elimination.

A semifinished (ingot to billet) mill yield of 81.6 percent was realized in the production of the foregoing billet products of the zirconium-treated steel, as compared to a yield of 60.9 percent for the untreated steel products. Increased yield resulted principally from decreased center segregation in the zirconium-containing steel.

These zirconium-containing steels exhibit machinabilities equal or superior to those of the zirconium-free machining steels.

Physical properties of representative table XI steels, after hot rolling to 15/16-inch rounds, are given in table XIII.

TABLE XIII

| Steel   | Percent Zr | 2% offset Y.S., p.s.i. | U.T.S., p.s.i. | Percent elongation in 2 inches |
|---------|------------|------------------------|----------------|--------------------------------|
| 52D524  |            | 55,050                 | 88,530         | 27.0                           |
| KX-0134 | .011       | 54,420                 | 89,870         | 27.0                           |
| KX-0135 | .014       | 57,420                 | 97,860         | 24.0                           |
| KX-0136 | .030       | 56,120                 | 93,610         | 25.0                           |

from which it will be seen that, in the range 0.014 to 0 percent zirconium, the steels investigated showed enhanced yield and tensile strengths with excellent retained ductility compared to the zirconium-free steels.

Macroexamination of the top three and the bottom ("billet from each of the table XI ingots revealed the presence of extensive visible center segregation and subsurface porosity in the untreated steel billets (from Ingot No. 2). Subsegregation and porosity was observed in the billets from Ingot No. 5 (0.011 percent Zr), while the billets from the higher ingots, Ingot No. 6 (0.014 percent Zr), No. 7 (0.030 percent Zr) and No. 8 (0.026 percent Zr) were found to be essentially free of visible segregation and subsurface porosity.

We have also found the above-described free-machining steels containing zirconium to be of greatly improved hot workability as compared to the same steels without the zirconium addition. Thus, usual mill practice with the 21×23 inch ingot above described is to (1) reduce the ingot, from an intermediate-sized article, e.g., to an 18½×20 inch cross section (2) reheat to the hot rolling temperature, and (3) thereafter roll the article to the form of a 2- to 3-inch square-section billet. Attempted direct rolling of the above-described zirconium-free gun barrel steels from the original ingot to 2½-inch billet form resulted in disintegration of such articles during rolling.

We have found, however, that the same steels, with the addition of at least about 0.015 percent zirconium, can be rolled without reheating, from ingots of, e.g., 19×22 inch cross section, directly to 2½-inch billets without any difficulty whatever, and, further, that such latter products have a high quality hot-rolled surface, free of seams, than do the prior steels even when the latter are subjected to intermediate heating.

We believe, but without being bound by this theory, that such improved hot workability of our new steels is due, at least in part, to the diminution or substantial elimination in the new steels of large sulfide inclusions and sulfur- and phosphorus-containing segregations. Thus, we have observed that, quite unexpectedly, the addition of at least about 0.015 percent zirconium to resulfurized and/or rephosphorized free-machining steels, such as the aforementioned gun barrel steel, results in large sulfides being broken up and dispersed substantially uniformly throughout the steel article. This ability of such zirconium additions to accomplish a dispersion of sulfide inclusions without any pronounced change in the morphology of inclusions, we believe to have improved both the hot-rolling characteristics of the steel ingots and the internal soundness and homogeneity (as shown by macro etch tests).

Further, phosphorus has a similar tendency to segregate with the sulfur in the steel. With the sulfur of sulfide inclusions dispersed, the phosphorus has also been dispersed with a concomitant improvement in properties of the steel.

As above described and shown, the aforementioned beneficial effects of zirconium are obtained by the addition of from about 0.015 to about 0.05 percent of that element. About 0.0 percent zirconium is a preferred upper limit of that element whereby the most significant benefits of the invention are obtained at lowest cost. Larger percentages of zirconium may be added within the limits prescribed by economics and/or interaction of these and other effects of zirconium upon the desired steel properties. Broadly, we contemplate the addition of zirconium up to about 0.15 percent for the purpose of

achieving the desired results herein taught. Greater amounts may be used to achieve supplemental results as may be desired.

The use of such zirconium additions is contemplated for any free-machining carbon or low alloy steel wherein the aforesaid newly discovered beneficial effects of such addition may be utilized with advantage. For example, free-machining steels containing segregation-prone elements as selenium or tellurium in supplement to or in place of sulfur are included within the scope of the invention.

Our steels preferably contain carbon in the range of about 0.10 to 0.60 percent together with silicon up to about 0.30 percent, preferably up to about 0.10 to 0.15 percent silicon. An adverse effect of silicon upon machinability becomes pronounced in steels having a carbon content below about 0.08 to 0.10 percent. Therefore, at the lower end of the carbon range, especially below about 0.14 percent carbon, silicon should be held at the low end of its range. In the case of such steels, the zirconium is preferably added as elemental zirconium metal, to avoid introduction of silicon, as in iron-silicon-zirconium alloys. Carbon is preferably held to 0.55 or 0.60 percent maximum, especially 0.45 to 0.55 percent, although special applications, requiring higher carbon up to 1.0 or 1.5 percent, may also benefit from the principles of the invention.

Broadly, manganese may be present in our improved free-machining steels in amount from 0.30 to 1.65 percent. Manganese contents above the minimum, e.g., at least about 0.70 percent, are preferred however, especially when sulfur is in the high end of its range.

In view of the ready combination of zirconium with oxygen in molten steel, it is highly desirable that the steels be at least partially deoxidized or "killed" prior to or along with the addition of zirconium. We have found zirconium utilization efficiencies of 50 to 80 percent to be readily achievable in the production of semikilled steels such as the gun barrel steels exemplified above, wherein the zirconium additions were made, after silicon blocking, to either ladle or mold.

It is to be understood that the foregoing description and specific examples are illustrative of the principles of the invention, and that various modifications and additions may be

made thereto by those skilled in the art without departing from the spirit and scope of the invention as set forth in the following claims.

We claim:

5 1. An improved free-machining semikilled gun barrel steel consisting essentially of, by weight percent,

|    |            |                                            |
|----|------------|--------------------------------------------|
| 10 | carbon     | 0.30 to 0.45%                              |
|    | manganese  | 0.70 to 1.0%                               |
|    | silicon    | 0.10% maximum                              |
|    | sulfur     | 0.08 to 0.15%                              |
|    | phosphorus | 0.07 to 0.12%                              |
|    | zirconium  | 0.015 to 0.07%                             |
|    | iron       | balance, except for incidental impurities, |

15 15 said steel being characterized by providing articles of improved chemical and structural homogeneity, enhanced hot workability, hot rolled surface quality, superior hardness uniformity and increased yield and tensile strengths as compared to the zirconium-free steel.

20 2. A steel in accordance with claim 1, wherein the maximum zirconium content is 0.05 percent.

25 3. A steel in accordance with claim 2, wherein the steel contains up to about 0.20 percent chromium.

4. A method of producing free-machining resulfurized and 25 rephosphorized carbon steel articles of improved chemical and microstructural homogeneity and enhanced hot workability, comprising partially killing a molten steel containing carbon in an amount from 0.30 weight percent to 0.45 weight percent, sulfur in an amount from 0.08 weight percent to about 0.15 weight percent and phosphorus in an amount from 0.07 weight percent to about 0.12 weight percent, and adding thereto a zirconium-containing material in amount sufficient to provide the steel with a zirconium content of at least about 0.015 weight percent.

30 5. A method in accordance with claim 4, wherein the steel contains from 0.70 to 1.0 percent manganese, and up to 0.10 percent silicon.

35 6. A method in accordance with claim 4, wherein the zirconium content of the steel is limited to a maximum of 0.07 percent.

\* \* \* \* \*

UNITED STATES PATENT OFFICE  
CERTIFICATE OF CORRECTION

Patent No. 3,634,073 Dated January 11, 1972

Inventor(s) John G. Cutton, et al.

It is certified that error appears in the above-identified patent and that said Letters Patent are hereby corrected as shown below:

Column 2, line 32, after "U.S.", insert -- Reissue -- .  
Column 6, line 63, change "of" to read -- or -- . Column 7,  
line 26, change "out" to read -- our -- .

Signed and sealed this 31st day of October 1972.

(SEAL)

Attest:

EDWARD M.FLETCHER,JR.  
Attesting Officer

ROBERT GOTTSCHALK  
Commissioner of Patents